

## 1

3,337,651

**MODIFICATION OF STEREOREGULAR POLYOLEFINS WITH POLYMERIC COMPOSITIONS**

Jack J. Press, 1218 E. Laurelton Parkway,

Teaneck, N.J. 07666

No Drawing. Filed Sept. 28, 1965. Ser. No. 491,055

6 Claims. (Cl. 260—895)

The invention described herein may be manufactured and used by or for the Government of the United States of America for governmental purposes without the payment of any royalties thereon or therefor.

This application is a continuation-in-part of my co-pending application Serial Number 400,611, filed Sept. 30, 1964, which is a continuation-in-part of application Serial Number 113,972, now abandoned.

The invention relates to stereoregular polyolefins. More particularly, this invention relates to polymeric compositions having improved affinity for dyes, said compositions containing a major amount of stereoregular polyolefins.

It is known that polyethylene is vastly unsuitable for the production of textile fibers due to the relatively poor properties imparted to the product. For one thing, a staple polyethylene fiber will not hold a crimp and this is necessary for textile processing. For another, it is useless to make a textured or stretched yarn from a continuous polyethylene filament because the characteristics imparted to the yarn are not maintained during weaving, dyeing, or ordinary use. Further, the material from which a fabric is made must be thermally stable before it may be subjected to ordinary use. It must not have a relatively low melting point, and the final fabric must not have a high degree of heat sensitivity, nor relatively soft mechanical properties at elevated temperatures. However, the thermal properties of a polyethylene fabric are such that it is impossible to subject it to ordinary ironing without physically damaging the fabric and it has been found to shrink in the conventional dryer. As is apparent from the foregoing, polyethylene cannot be utilized in the manufacture of everyday fabrics for ordinary use.

In recent times, it has been found that certain linear crystalline hydrocarbon polymers containing stereoregular macromolecules and having melting points between 150° and 300° C. can be used for the production of textile fibers without the inherent difficulties encountered with the use of polyethylene polymers for this purpose. Aside from melting point differences, polypropylene with a tertiary carbon and a methyl side chain, crystallizes differently and has a much higher resilience and elasticity. These properties are essential in generally useful textile fiber. Further, polymers of olefinic hydrocarbons containing stereoregular macromolecules, such as polypropylene, polymethylpentene, and polymethylbutene, offer considerable advantages in the production of fibers, particularly because of their good mechanical properties and light weight. However, such polymers have not been satisfactory because of their poor affinity for dyes, this poor affinity being due to the particular chemical nature of such polyolefinic hydrocarbons.

Many processes have been proposed in order to improve the affinity of such polyolefinic hydrocarbons for dyes, such as the addition of soluble solid substances to the molten polyolefin before spinning. The addition of basic substances facilitates dyeing with acid dyes, whereas the addition of acid substances favors dyeing with basic dyes. However, such processes have not been completely satis-

## 2

factory because soluble modifiers interfere with crystallization, impair strength and thermal stability, and are not sufficiently available in the amorphous regions where dyeing takes place.

It has also been proposed to increase the affinity of dyes for polyolefin fibers by grafting monomers onto the fibers after subjecting the fibers to a preliminary peroxidation or to high energy radiation. When such processes are applied to the polyolefin after it is in filamentary form the surface properties of the grafted fibers are considerably modified and the dye receptivity is improved. However, when such processes are applied to highly crystalline filaments, any grafting onto the preformed fibers takes place only at the surface. Therefore, subsequent dyeing is limited to the surface portion of the fiber and the dye does not penetrate inside the fiber.

It is therefore an object of this invention to provide a polymeric composition having improved affinity for dyes devoid of all the difficulties of the prior art.

In my co-pending application, Serial No. 400,611, filed Sept. 30, 1964, I describe a class of modified stereoregular polyolefins having increased affinity for dyes and other polar substances comprising a matrix of a stereoregular polyolefin taken from the group consisting of polypropylene, polymethylpentene and polymethylbutene, said matrix of polyolefin having dispersed therein between about 2 and 20% of a modifying polymer which is hydrophilic, non-soluble in the polyolefin and fusible at a temperature not exceeding the temperature of processing of the polyolefin (150° C. to 350° C.), said modifying polymer being selected from the group consisting of alkylene oxide polymers having molecular weights between 100,000 and 5,000,000; poly N-vinyl pyrrolidone; poly N-vinyl morpholine; and poly N-vinyl oxazolidinone.

However, the above heterocyclic modifiers only show poor to fair uniformity of dispersion in the stereoregular polyolefin.

This invention relates to stereoregular polyolefins, modified with chemically substituted heterocyclic polymers, having an affinity for dyes and other polar substances to a degree at least equal to that shown in the above co-pending application, but with improved uniformity of dispersion. The polymeric compositions of this invention comprise a matrix of stereoregular polyolefin taken from the group consisting of polypropylene, polymethylpentene, and polymethylbutene, said matrix having dispersed therein between 2 and 20% of a second, hydrophilic, non-soluble, fusible and partially substituted polymeric composition, said second substituted polymeric composition consisting of one of the following, viz:

(a) 50 to 98 mole percent of N-vinyl methyl oxazolidinone and 2 to 50 mole percent of N-vinyl-R-oxazolidinone where R is an alkyl, aryl, alkaryl, or alkoxy group having 4 to 30 carbons;

(b) 50 to 98 mole percent of N-vinyl morpholinium and 2 to 50 mole percent of N-R quaternary N-vinyl morpholinium wherein R is an alkyl, aryl, alkaryl, or alkoxy group having 4 to 30 carbons;

(c) 50 to 98 mole percent of N-vinyl pyrrolidone and 2 to 50 mole percent of R-4-vinylamino butanamide wherein R is an alkyl, aryl or alkaryl group having 4 to 30 carbons;

(d) 50 to 98 mole percent of N-vinyl pyrrolidone and 2 to 50 mole percent of R-4-vinylamino butanoate wherein R is an alkyl, aryl, alkaryl group having 4 to 30 carbons; and

(e) 50 to 98 mole percent of N-vinyl pyrrolidone and 2 to 50 mole percent of N-vinyl-R-oxazolidinone wherein R is an alkyl, aryl, alkaryl or alkoxy group having 4 to 30 carbons.

The stereoregular polyolefins which may be used within the concept of this invention include isotactic and syndiotactic polyolefins. These materials are usually made by utilizing stereo-specific catalysts which give polymers which are substantially linear and which develop a high degree of crystallinity.

Within this concept, for improved dispersibility, 2 to 50% of the monomeric units of the heterocyclic polymer making up the second polymeric composition are substituted by the introduction of substituents having at least one alkyl, alkaryl, aryl or alkoxy group with 4 to 30 carbons. There is no significant reduction in melting point or improvement in dispersibility when less than 2% of the heterocyclic polymer are substituted. However, if more than 50% of the heterocyclic polymer is substituted, this will result in excessive softening of the heterocyclic polymer, increased solubility in the polymer, and the need for increased addition of the heterocyclic polymer in order to obtain the level of modifier needed for dyeability and printability. Excessive solubility in the polyolefin tends for excessive sweating out and separation of the modified polymer substituents. However, the latter material may be easily removed from the polyolefin by laundering and solvents.

I prefer to stay below 25% level of substitution of the heterocyclic polymer, when the substituents have 12 or more carbon atoms. This is because the latter type substituents have a more pronounced effect on softening and solubility of the material in the polyolefin. The degree of substitution should be low enough to insure that the substituted heterocyclic polymer remains hydrophilic and soluble or dispersible in water or an oxygenated solvent. The substituted polymer should also be non-soluble in the polyolefin and fusible at a temperature not exceeding the temperature of processing of the polyolefin (150 to 350° C.).

The substitution of the heterocyclic polymer may take place either prior to, during, or after polymerization of the heterocyclic polymer. This can be accomplished by techniques known in the art such as substitution on a carbon of the heterocyclic ring, quaternization of the tertiary N-alkenyl group, or by hydrolysis of the ring amide and reaction of the liberated carboxy or amine groups with an alcohol, acid, or amine group having 4 to 30 carbons. The above would include substitution on the ring carbon of N-vinyl oxazolidinone, quaternization of N-vinyl morpholine, and partial hydrolysis of the ring amide of N-vinyl pyrrolidone and reaction of the liberated carboxy groups with fatty amines or alcohols.

The following examples will illustrate the utility of the present composition:

#### Example I

(1) Each of the polymers, substituted or not, was ground to a powder (50 to 200 mesh), mixed with a given proportion of a powdered (50 to 200 mesh) commercial isotactic polypropylene (molecular weight of 350,000; melting point of about 170° C.; melt flow index of 3; and isotacticity of 95%) and formed into a disc in the following manner.

(2) The powder of each sample was spread uniformly in a circular shouldered Pyrex glass dish with an inside diameter of 4 inches. The dishes were then covered by an inner nesting circular shouldered Pyrex glass dish with a bottom outer separation rib projecting downwardly about 0.05 inch. The assembly weighted with a preheated 5 pound weight was then placed in an oven at 250° C. for 6 to 15 minutes. Then the weight was removed and the assembly was placed in a refrigerator at about 4° C. to cool. The assembly dishes were then separated to give a fused disc and judged for uniformity of dispersion.

(3) The disc was then cut radially into 6 equal sec-

tions and re-fused four times, at which time, the disc was again judged for uniformity of dispersion.

(4) The uniformity was rated as very poor—no apparent dispersion, poor—slight dispersion, fair—moderate dispersion, good—almost complete dispersion, and excellent—complete dispersion.

TABLE I

The following modifier combinations were formed into discs in the manner set forth above in an amount between 10 and 20% based on the amount of polypropylene utilized.

- (1A) (blank) poly N-vinyl methyl oxazolidinone
- (1B) 50% (1A)\*—50 mole percent N-vinyl butyl oxazolidinone
- (1C) 75% (1A)\*—25 mole percent N-vinyl butyl oxazolidinone
- (1D) 85% (1A)\*—15 mole percent N-vinyl octyl oxazolidinone
- (1E) 90% (1A)\*—10 mole percent N-vinyl lauryl oxazolidinone
- (1F) 98% (1A)\*—2 mole percent N-vinyl lauryl oxazolidinone
- (1G) 75% (1A)\*—25 mole percent N-vinyl tolyl oxazolidinone
- (1H) 90% (1A)\*—10 mole percent N-vinyl nonylbenzyl oxazolidinone
- (1I) 75% (1A)\*—25 mole percent N-vinyl butoxy oxazolidinone

30 \*Monomeric units in polymer.

The discs formed above were then judged for uniformity after one and five fusing or molding cycles as follows:

35

| 40 | Modifier | Percent Modifier* | Dispersion Uniformity |                  |
|----|----------|-------------------|-----------------------|------------------|
|    |          |                   | One Mold Cycle        | Five Mold Cycles |
| 45 | 1A       | 2                 | Fair.....             | Fair-good.       |
|    | 1A       | 5                 | do.....               | Fair.            |
|    | 1A       | 10                | Poor.....             | Poor-fair.       |
|    | 1A       | 20                | Very poor.....        | Poor.            |
|    | 1B       | 5                 | Good.....             | Excellent.       |
|    | 1B       | 20                | Fair.....             | Good.            |
|    | 1C       | 2                 | Good.....             | Excellent.       |
|    | 1C       | 10                | do.....               | Do.              |
|    | 1C       | 20                | Fair.....             | Good.            |
|    | 1D       | 5                 | Good.....             | Excellent.       |
|    | 1D       | 10                | do.....               | Do.              |
|    | 1E       | 10                | do.....               | Do.              |
|    | 1F       | 10                | Fair.....             | Good.            |
|    | 1G       | 5                 | Good.....             | Excellent.       |
|    | 1H       | 5                 | do.....               | Do.              |
|    | 1I       | 5                 | do.....               | Do.              |

55 \*Percent by weight of modifier in polyolefin.

#### Example 2

60 In accordance with the general procedure set forth in Example 1, I prepared polypropylene discs having various modifier combinations incorporated therein as follows:

| 65 | Discs: | TABLE 2                              |                                                                    |                                                                    |                                                                   |                                                                   |
|----|--------|--------------------------------------|--------------------------------------------------------------------|--------------------------------------------------------------------|-------------------------------------------------------------------|-------------------------------------------------------------------|
|    |        | (2A) (blank)—poly N-vinyl morpholine | (2B) 75%* (2A)—25 mole percent octyl N-vinyl morpholinium chloride | (2C) 90%* (2A)—10 mole percent octyl N-vinyl morpholinium chloride | (2D) 75%* (2A)—25 mole percent butyl N-vinyl morpholinium sulfate | (2E) 90%* (2A)—10 mole percent butyl N-vinyl morpholinium sulfate |
| 70 |        |                                      |                                                                    |                                                                    |                                                                   |                                                                   |

75 Footnote at end of table.

TABLE 2—Continued

- (2F) 90%\* (2A)—10 mole percent stearyl N-vinyl morpholinium chloride  
 (2G) 98%\* (2A)—2 mole percent stearyl N-vinyl morpholinium chloride  
 (2H) 75%\* (2A)—25 mole percent benzyl N-vinyl morpholinium chloride  
 (2I) 90%\* (2A)—10 mole percent benzyl N-vinyl morpholinium chloride  
 (2J) 75%\* (2A)—25 mole percent butoxy N-vinyl morpholinium chloride

\*Monomeric units in polymer.

The discs above were then judged for uniformity of dispersion after one and five molding cycles and the results were set forth below:

RESULTS 2

| Modifier | Percent Modifier | Dispersion Uniformity |                  |
|----------|------------------|-----------------------|------------------|
|          |                  | One Mold Cycle        | Five Mold Cycles |
| 2A       | 5                | Fair                  | Fair             |
| 2A       | 20               | Very poor             | Poor             |
| 2B       | 5                | Good                  | Excellent        |
| 2C       | 20               | Fair                  | Good             |
| 2C       | 5                | Good                  | Excellent        |
| 2D       | 10               | Fair                  | Do               |
| 2D       | 5                | Good                  | Do               |
| 2D       | 20               | Fair                  | Good             |
| 2E       | 5                | Good                  | Excellent        |
| 2E       | 10               | Fair                  | Do               |
| 2F       | 5                | Good                  | Do               |
| 2F       | 10               | do                    | Do               |
| 2G       | 5                | do                    | Do               |
| 2H       | 5                | do                    | Do               |
| 2I       | 5                | do                    | Do               |
| 2J       | 5                | do                    | Do               |

## Example 3

In accordance with the general procedure set forth in Example 1, I prepared polypropylene discs having various modifier combinations incorporated therein as follows:

TABLE 3

## Discs:

- (3A) (blank)—100% poly N-vinyl pyrrolidone  
 (3B) 50% (3A)—50 mole percent N-butyl 4-vinyl-amino butanamide  
 (3C) 75% (3A)—25 mole percent N-butyl 4-vinyl-amino butanamide  
 (3D) 90% (3A)—10 mole percent N-butyl 4-vinyl-amino butanamide  
 (3E) 75% (3A)—25 mole percent octyl 4-vinyl-amino butanoate  
 (3F) 90% (3A)—10 mole percent octyl 4-vinyl-amino butanoate  
 (3G) 98% (3A)—2 mole percent octyl 4-vinyl-amino butanoate  
 (3H) 90% (3A)—10 mole percent lauryl 4-vinyl-amino butanoate  
 (3I) 98% (3A)—2 mole percent lauryl 4-vinyl-amino butanoate  
 (3J) 75% (3A)—25 mole percent N-benzyl 4-vinyl-amino butanamide  
 (3K) 90% (3A)—10 mole percent laurylbenzyl 4-vinylamino butanamide  
 (3L) 75% (3A)—25 mole percent N-vinyl tolyl-pyrrolidone  
 (3M) 90% (3A)—10 mole percent N-vinyl octa-benzylpyrrolidone  
 (3N) 75% (3A)—25 mole percent N-vinyl butyl-pyrrolidone

The discs made with the modifier combinations set forth in Table 3 were then judged for uniformity of dispersion after one and five molding cycles and the results were set forth below:

RESULTS 3

| 5  | Modifier | Percent Modifier | Dispersion Uniformity |                  |
|----|----------|------------------|-----------------------|------------------|
|    |          |                  | One Mold Cycle        | Five Mold Cycles |
| 3A |          | 2                | Fair                  | Fair             |
| 3A |          | 5                | Poor to fair          | Do               |
| 3A |          | 10               | Poor                  | Do               |
| 3A |          | 20               | Very poor             | Poor             |
| 3B |          | 20               | Fair                  | Excellent        |
| 3C |          | 10               | Good                  | Do               |
| 3D |          | 10               | Fair                  | Do               |
| 3D |          | 5                | Good                  | Do               |
| 3E |          | 20               | Fair                  | Do               |
| 3E |          | 10               | Good                  | Do               |
| 3F |          | 10               | Fair                  | Do               |
| 3F |          | 5                | Good                  | Do               |
| 3G |          | 5                | Fair                  | Good             |
| 3G |          | 2                | Good                  | Excellent        |
| 3H |          | 10               | do                    | Do               |
| 3I |          | 5                | do                    | Do               |
| 3I |          | 2                | do                    | Do               |
| 3J |          | 5                | do                    | Do               |
| 3K |          | 5                | do                    | Do               |
| 3L |          | 5                | do                    | Do               |
| 3M |          | 5                | do                    | Do               |
| 3N |          | 5                | do                    | Do               |

25 In all dye tests with discs prepared in accordance with the procedures of Examples 1 to 3, the stereoregular polyolefinic discs modified with chemically substituted heterocyclic polymers gave more uniform results in comparison with the discs which were only modified with an 30 unsubstituted polymer.

Many alternate methods of combining my modifier combinations with polyolefins are readily available. They may be combined during formation of the polymeric modifier or during actual polymerization of the olefin, 35 with or without melting. They may be added to freshly polymerized polyolefin, which is still in solution in a suitable solvent, in the powdered form, or as a solution in a compatible solvent, or merely as a dispersion. They may be added to the polyolefin during precipitation, 40 washing, neutralizing or compounding of the freshly prepared polyolefin prior to drying. This may be accomplished by adding the modifier as a powder or as a solution which is a non-solvent for the polyolefin.

The modifiers combinations may also be melt mixed 45 during processing or blending of the polymer prior to use in extension of fiber, film, coating or plastic. It may also be added as a liquid or powder to finely ground or micronized polyolefin polymers and then melt dispersed in situ during hot dip or spray coating or during spreading and heat coating operation. They may be incorporated in polyolefin solutions or emulsion and then applied to surfaces with or without heating.

The level of addition of the modifiers heretofore listed 55 should be between 2 and 20% of the weight of the overall composition. If less than 2% is utilized, significant improvement will not be achieved in dyeability. If an amount greater than 20% is added to the polyolefin, many of the physical properties of the final product, such as fiber or film, are adversely affected. These include loss of strength and a lower resistance to repeated flexing.

Under the present concept, I prefer hydrophilic polymeric modifiers which may be soluble to either water or an oxygenated solvent but which are not soluble in the polyolefin. I do prefer modifiers which are fusible and can be dispersed in the polyolefin.

Prior experience with comparatively less hydrophobic fiber forming polymers, such as polyacrylonitrile polymers and polyamides, have shown that the use of hydrophilic, water soluble or dispersible, modifiers is impractical. Mainly, because excessive amount of the modifier are leached out in scouring and dyeing processes. Surprisingly, I have found that my hydrophilic polymeric modifiers, when melt dispersed in the more hydrophobic polyolefin, have good dispersion stability and are not susceptible to leachage.

I have found that at comparatively low levels of addition, my modifiers confer good dyeability on the polyolefin without the necessity for costly and sometimes impractical post treatments.

My hydrophilic modifiers must be fusible with the polyolefin. This is necessary for the formation of a continuous network of modifier throughout the polyolefin in order to permit dye penetration and efficient coordination of the dye and modifier throughout the film or fiber.

The use of a non-fusible cross-linked modifier, which results in poor dispersion, is ineffectual. The required modifier network in such a case cannot be formed and the discrete, separate particles are surrounded by unmodified areas within the polyolefin matrix. As a result, dyeing is limited to the fiber surface and the dye cannot penetrate into the interior of the fiber where it is most desired.

It is generally recognized that dyeing takes place almost entirely in the more open and readily accessible amorphous areas. When a soluble modifier is utilized, it is usually spread throughout the amorphous and crystalline areas of the polyolefin. As a result, the modifier in the crystalline areas is not available for improvement in dyeability. It also interferes with crystallization and adversely affects strength and thermal stability. However, my non-soluble, hydrophilic, polymeric modifiers are not sufficiently compatible to be a part of the more uniform and denser crystalline areas. It appears to concentrate in the more amorphous areas where it is necessary for dyeability. It has also been found that an increase in molecular weight of my modifiers, further reduces compatibility with stereoregular polyolefins and promotes concentration of the modifier in the more amorphous regions where it may improve the dyeability of the polyolefinic matrix.

Obviously, many modifications and variations of the present invention are possible in the light of the above teaching. For instance, the modifiers of this invention may be used to increase the opacity and the affinity of the polyolefin for finishes. They may also be used to improve the printable of the polyolefin, increase the adhesion of the polyolefin to other materials, or to reduce the overall static propensity of the final product. It is therefore to be understood that within the scope of the appended claims, the invention may be practiced otherwise than as specifically described.

I claim:

1. A polymeric composition having improved affinity for dyes comprising:

a matrix of stereoregular polyolefin taken from the group consisting of:

polypropylene,  
polymethylpentene, and  
polymethylbutene,

said matrix having dispersed therein between 2 and 20 percent of a second, hydrophilic, non-soluble, fusible and partially substituted polymeric composition,

said second polymeric composition being selected from the group consisting of:

(a) 50 to 98 mole percent of N-vinyl methyl oxazolidinone and 2 to 50 mole percent of N-vinyl-R-oxazolidinone wherein R is selected from the group consisting of an alkyl, aryl, alkaryl or an alkoxy group having 4 to 30 carbons;

(b) 50 to 98 mole percent of N-vinyl morpholinium and 2 to 50 mole percent of N-R-quaternary N-vinyl morpholinium wherein R is selected from the group consisting of an alkyl, aryl, alkaryl, or an alkoxy group having 4 to 30 carbons;

(c) 50 to 98 mole percent of N-vinyl pyrrolidone and 2 to 50 mole percent of R-4-vinylamino butanamide wherein R is selected from the group consisting of alkyl, aryl, or an alkaryl group having 4 to 30 carbons;

(d) 50 to 98 mole percent of N-vinyl pyrrolidone and 2 to 50 mole percent of R-4-vinylamino butanoate wherein R is selected from the group consisting of an alkyl, aryl, or an alkaryl group having 4 to 30 carbons; and

(e) 50 to 98 mole percent of N-vinyl pyrrolidone and 2 to 50 mole percent of N-vinyl-R-pyrrolidone wherein R is selected from the group consisting of an alkyl, aryl, alkaryl or alkoxy group having 4 to 30 carbons.

2. The composition of claim 1 wherein said second partially substituted polymeric composition is 50 to 98 mole percent of N-vinyl methyl oxazolidinone and 2 to 50 mole percent of N-vinyl-R-oxazolidinone wherein R is selected from the group consisting of an alkyl, aryl, alkaryl or an alkoxy group having 4 to 30 carbons.

3. The composition of claim 1 wherein said second partially substituted polymeric composition is 50 to 98 mole percent of N-vinyl morpholinium and 2 to 50 mole percent of N-R-quaternary N-vinyl morpholinium wherein R is selected from the group consisting of an alkyl, aryl, alkaryl, or an alkoxy group having 4 to 30 carbons.

4. The composition of claim 1 wherein said second partially substituted polymeric composition is 50 to 98 mole percent of N-vinyl pyrrolidone and 2 to 50 mole percent of R-4-vinylamino butanamide wherein R is selected from the group consisting of an alkyl, aryl, or an alkaryl group having 4 to 30 carbons.

5. The composition of claim 1 wherein said second partially substituted polymeric composition is 50 to 98 mole percent of N-vinyl pyrrolidone and 2 to 50 mole percent of R-4-vinylamino butanoate wherein R is selected from the group consisting of an alkyl, aryl or an alkaryl group having 4 to 30 carbons.

6. The composition of claim 1 wherein said second partially substituted polymeric composition is 50 to 98 mole percent of N-vinyl methyl pyrrolidone and 2 to 50 mole percent of N-vinyl-R-pyrrolidone wherein R is selected from the group consisting of an alkyl, aryl, alkaryl, or alkoxy group having 4 to 30 carbons.

No references cited.

MURRAY TILLMAN, Primary Examiner.

D. J. BREZNER, Assistant Examiner.